

June 23, 1936.

L. T. TROLAND

2,044,864

METHOD OF MAKING LIGHT SENSITIVE FILMS

Filed May 23, 1930

2 Sheets-Sheet 1



June 23, 1936.

L. T. TROLAND

2,044,864

METHOD OF MAKING LIGHT SENSITIVE FILMS

Filed May 23, 1930

2 Sheets-Sheet 2

Fig. 5



inventor  
Leonard T. Troland,  
By Robert Gusman, Woodbury.  
Attys.

## UNITED STATES PATENT OFFICE

2,044,864

## METHOD OF MAKING LIGHT SENSITIVE FILMS

Leonard T. Troland, Cambridge, Mass., assignor,  
by mesne assignments, to Technicolor, Inc.,  
New York, N. Y., a corporation of Delaware

Application May 23, 1930, Serial No. 454,973

## 15 Claims.

(Cl. 95—7)

This invention relates to photographic positive emulsions or films,—especially for use in cinematography and cinematographic reproductions (as for example by the imbibition process 5 of dyeing a matrix film and printing blank films therefrom) in color or in black and white and to a method of preparing and using the same.

In the art of making photographic images to represent views of objects which present wide 10 ranges of light intensity or contrast (i. e., corresponding to high-lights, half or middle tones, and shadows) it is important that the appropriate gammas or density gradations shall be attained therein, and shall be consistently obtainable 15 throughout the entire range of intensities and corresponding densities which may occur in any given instance. In photographic images which are formed in the usual light sensitive silver emulsions or films such density variations are 20 produced by the relative densities of reduced silver granules and/or depths of penetration of the exposure light into the emulsions, effective to form such metallic silver granules—which correspond in a general way to the logarithm of 25 the relative intensities and/or depths of penetration of the exposure light, respectively.

In the sensitive silver emulsion films as ordinarily prepared, however, it is found that such silver images are produced primarily by the ultra 30 violet, violet or blue component of the exposure light to which the emulsions usually used are predominantly sensitive and accordingly the emulsions present a relatively narrow or limited range of sensitivity, with respect to the spectral 35 composition of the light to which they are exposed. Moreover, in such images there is a tendency for the gradations of density or gamma in the higher ranges of density in the developed film to be abnormally low, although the intermediate 40 ranges of densities may be substantially correct in this respect and correspond accurately to the relative intensities of the light to which the emulsion has been exposed.

In other words, if the density of the metallic silver—or depth to which the exposure light has 45 penetrated the emulsion and affected the formation of granules of silver salt contained therein,—be plotted against the logarithm of increasing intensities or time of the exposure light, a curve 50 of the characteristics indicated in Fig. 4 will usually be obtained. As shown by this curve the density increases only gradually in the lower and upper portions of the curve while in the intermediate range the density gradation or gamma is

more nearly directly proportional to the logarithm of the intensity.

It is therefore desirable to extend the range 5 of densities obtainable in the photographic emulsion and to obtain throughout said range density gradation or contrast gradients more accurately to correspond to the range of intensities and relative contrasts presented by the exposure light. It is also desirable under special circumstances, to 10 vary at will and independently the relative contrasts in regions of different intensities.

Furthermore, if photographic images as heretofore produced in the manner described are 15 formed in physical relief (as by dissolving and removing the undeveloped portions of the gelatine emulsion) the image which is left presents a relief, the thicknesses of which substantially correspond to the density of the silver image, while the contours or relative thicknesses represent the 20 gradations of density or contrast. In such relief images, however, the same limitations of range 25 of sensitivity to the exposure light and failure of correlation of densities are present as are manifested by the original silver image. Thus, the higher relief contours (densities) may present 30 lower gradients or slopes than the intermediate contours; and in practice such gradient may be reduced by the dissolving operation in these extreme parts of the relief more than in the intermediate portion.

Accordingly, in both types of photographic images i. e. whether produced by densities of metallic silver or depth of penetration of the exposure light into the developed emulsion or by the contours in the gelatine relief, the image may 35 be deficient in gamma (i. e., density gradient or relief contour slope) in one or more regions of variation of intensity of the exposure light; and also limited with respect to the range of densities or thicknesses of relief which may be relied 40 upon for accurate contrast reproduction.

Moreover, when films containing such images (and especially gelatine relief images which are the more commonly employed for the purpose) are wet with a solution of a dye which they selectively adsorb and/or absorb and the dye wet surfaces then applied to a blank film for the imbibition transfer of the absorbed dye image to the blank, it is found that the contrast gradients and ranges of contrast obtained in the thus 50 printed dye image are still further reduced. In such cases, the dye absorbed and transferred by the higher portions of the relief image, forms dye images characterized by low gamma or contrast. Furthermore, such disproportionate absorption 55

of dye by the matrix film image and/or transfer of the same by imbibition to the blank film may occur even though the matrix film were substantially correct with respect to its contrast 5 gradients (or contours) throughout the range of light intensities represented thereby. This result may be due for example (1) to disproportionate absorption or adsorption of dye in the several areas of the matrix (2) disproportionate transfer 10 of the dye therefrom and/or disproportionate imbibition by the blank film, or (3) permanent retention of a part of the dye by the matrix film. Such disproportionate formation of the dye image, resulting in loss of contrast or gamma, 15 occurs primarily in the areas of high densities or light intensities but may occur anywhere in the range of densities—low, medium or high.

It is therefore desirable and an object of this invention to effect an individual and independent 20 control of the several gammas (i. e., contrast gradients in the developed emulsion or relative contour gradients in the physical relief images) in each of the regions of the photographic image corresponding to the low, medium and high 25 ranges of light intensity in the exposure light. It is also an object to extend the aggregate range of light intensities which may be reproduced and throughout which such control of the gamma or contrast in the photographic image may be 30 effectuated. It is a further object so to control the effective gammas in the photographic image of a matrix film (for imbibition purposes) that the absorption and/or adsorption of a dye solution and transfer of the same by imbibition to 35 a blank film shall produce a dye image upon the latter characterized by a wider range of contrasts and by manifesting the desired gamma or contrast gradient throughout the range of light (color) intensities to be reproduced thereby. It 40 is also an object to vary at will (and independently) the relative contrasts in regions of different intensity. Other objects will appear from the following disclosure.

The invention includes briefly the preparation 45 of a photographically sensitive (silver) gelatine emulsion preferably by treating with one or more sensitizing agents to render the same sensitive to a broader spectral band of light (e. g., corresponding to three spectral zones) and also by 50 dyeing with three (or more) dyes which are severally characterized by being selectively absorptive of light waves in separate spectral zones (preferably distinct but possibly overlapping) 55 within the said sensitized band.

The emulsion thus formed is characterized by a wider range of sensitivity than the silver emulsions heretofore employed in positive printing. And moreover, by employing a composite light 60 (of widely varying intensities and comprising light waves in each of the three spectral zones selectively absorbed by the dyes) in exposing the same, the contrast gradients (or relief contours) corresponding to the regions of low, medium and high intensities of the exposure light may be independently controlled by the successive and selective absorption of light of said spectral colors, 65 respectively.

Preferably the light of shortest wave length 70 will be sharply absorbed (by the specific absorptive dye therefor) to produce the lower range of densities or reliefs and thereby also to accentuate the gradation of density or contours within this range. The exposure light of intermediate wave length may be less sharply absorbed (by the dye

specifically absorptive thereof) and hence penetrate the emulsion deeper, to produce the range of intermediate densities and/or reliefs. In this range the gradations of density or contrast are ordinarily sufficiently well reproduced; but in this range the use of selectively light-absorptive dye restrains the corresponding light waves of the exposure light to the development of the intermediate range of intensities and prevents their further penetration. A portion of the remaining 10 still less strongly absorbed light (usually of still longer wave length) is permitted to penetrate more deeply into the gelatine emulsion but, due to the action of the third dye, may not pass entirely through the film and hence is effectively 15 absorbed therein to form the photographic image in the region of high densities or reliefs, with gradations or contours, (accentuated still more than in the regions of low densities or reliefs) and hence provides the required contrast in this 20 range of light intensity.

The specific absorption of light effected in each spectral zone of the exposure light may be in such proportion to the sensitivity of the emulsion with respect to light waves of that zone as to 25 reduce the depth of penetration or thickness of relief produced by the penetration of the exposure light, to the absolute (and relative) degree required. Accordingly the density gradient or 30 relief contour produced, corresponding to each zone of light intensity in the exposure, may be controlled by controlling the ratio of the absorptivity of the dye to specific sensitivity of the film to the absorbed light, as may be desired.

For example, a silver emulsion may be rendered 35 sensitive to blue-green, green and yellow light (in addition to the normal sensitivity to blue light), thus presenting a relatively wide zone of spectral sensitivity (or to three separate spectral zones if desired). It may also be treated with 40 dyes which are selectively absorptive of blue, blue-green, green and yellow light, respectively. The dyes may be employed, severally, in appropriate amounts or concentrations in relation to the sensitivity of the emulsion to light of the 45 several spectral wave lengths, to correspond to and control the formation of the photographic image produced by the low, medium and high intensities of the exposure light. Thus a dye strongly absorptive of blue light may be employed 50 in a film to reduce the density of an image (or thickness of its relief) to be produced thereon by the blue zone of the exposure light to represent the low intensities of the exposure light, and the degree of reduction will be controlled by the 55 amount of dye used and varied within such range by the relative intensities of the (blue component of the) exposure light employed. Thus, the gamma or relative degree of density or thickness of the relief image produced may be controlled 60 by the relationship of the specific absorption characteristics of the dye to the sensitivity characteristic of the emulsion in this spectral range, and determined by the quality, time and intensity of the blue component of the exposure light to 65 which it is subjected.

Likewise, the blue-green and green components of the exposure light, to which the emulsion has been sensitized, may be selectively absorbed by the second dye and the depth of penetration or 70 thickness of the relief image formed thereby may be reduced. But it may, for example, be reduced less than the depth of penetration of the image or thickness of relief produced by the blue light,—thereby to produce a region of deeper penetra- 75

tion of the emulsion and a higher relief in the resulting image, consequent upon this component and corresponding to the intermediate range of intensities of the exposure light. The gamma or gradation of relief produced in this zone of the exposure light will likewise be controlled by the relationship of the sensitizing and absorptive values of the reagents, in conjunction with the variations in intensities of the exposure light.

10 The third (e. g. greenish-yellow) component of the exposure light (to which the emulsion has been sensitized) may also be selectively absorbed by the presence of the third dye and the depths of penetration (or thicknesses of the relief image) formed thereby likewise somewhat reduced. But the degree of reduction of penetration in this zone may be relatively slight so as to permit deep penetrations of the emulsion by this component of the exposure light (limited only by the thickness of the film) thus to produce the high reliefs in the resulting photographic image and sharper contrast or contour gradients corresponding to the higher range of intensities of the exposure light.

25 In the above example, the positive film emulsion *f* (shown in section) according to the invention is throughout its thickness sensitive to blue, green and yellow light (that is, isochromatic in contradistinction to the positive emulsion normally used) and, likewise throughout its thickness, selectively absorptive of light in three zones in the blue, green and yellow regions of the spectrum. This absorption is, according to the invention, stepped in such a manner that substantially all blue exposure light is absorbed within depth *b* next to the light entrant side of the emulsion.

30 The absorption in the green zone is less strong, so that green printing light penetrates depth *g*. The absorption of yellow printing light is still less intensive, so that the latter penetrates depth *y*, that is, substantially the entire emulsion.

35 It will now be evident what happens when emulsion *f* is exposed to a record to be reproduced, for example a negative *n* represented by developed silver wedge *w*. The printing light contains at least the blue, green and yellow ranges indicated by rays *B*, *G*, and *Y*, but may be white, for obvious reasons. The highly absorbed blue printing light is exhausted within region *b*, and the exposure effected by it can be indicated by curve *L* representing the low intensities or high light portions of the positive, within sector *l* of the wedge. Similarly, the green light affects the medium intensity record *M* corresponding to region *m* and the yellow light the high intensity or shadow record *H*, corresponding to region *h* of the negative. Hence, the shape of the density exposure curve (or the contrast characteristic) 40 of the total record can be controlled and adjusted by substantially independently controlling the exposure within each of three depths *b*, *g*, *y*. The contrast control within each independent 45 contrast zone or band as well as the depth of penetration for each band can be controlled by adjusting sensitivity, absorption and printing light intensity for that band, zone or depth of penetration.

50 In the embodiment described, the gelatine portions above lines *L*, *M*, *H* would be dissolved or etched off, so that the resulting cross section of the relief reproduction of wedge *w* indicates directly the exposure control in the three depths, zones or contrast bands.

55 A typical example of the practical application

of the invention will be described with reference to a film of light sensitive silver emulsion, sensitized with respect to three spectral zones of light and rendered selectively absorptive of light in said zones by treatment with appropriate dyes, reference being made to the accompanying drawings in which:

Fig. 1 contains graphs of the individual spectral absorption values of the particular dyes in the concentrations employed, as ordinates, 10 against wave lengths of light as abscissae;

Fig. 2 contains a like graph (E) of the composite absorption values of the dyes employed and also a corresponding graph (F) showing the composite spectral sensitivity of the film; 15

Fig. 3 represents the cumulative penetrations or reliefs of an image resulting from exposure of the sensitized and dyed film of Fig. 2 to increasing intensities of exposure light and the gammas obtained in the low medium and high 20 intensity regions, respectively, in accordance with this invention;

Fig. 4 represents the usual graph or relief of an image resulting from exposure of an ordinary sensitive gelatine emulsion to increasing intensities of exposure light; and 25

Fig. 5 is a diagram explaining the new method and including a section through an emulsion forming an embodiment of the invention.

In Fig. 1, the graphs indicate the spectral absorption value of (A) tartrazine, (B) rose bengal, (C) acid magenta, (D) erythrosine components of the dye solution employed (given below) plotted in terms of the factor:

$$\log_{10} \frac{\text{Transmitted light}}{\text{Incident light}}$$

35

as ordinates and spectral wave lengths as abscissae.

In Fig. 2 the graph E represents, in the same 40 manner, the composite effects of the several dyes, while graph F indicates the spectral sensitivity of the film as sensitized primarily by silver halide in the region F', and by rose bengal and/or erythrosine in the region F''. The latter dye or 45 sensitizer develops an excessive sensitivity to light in the zone between 550 and 620. Consequently, by its addition to the emulsion there is an overcorrection and extension of sensitivity 50 in these spectral zones. This may be partially offset or neutralized by the use of a filter (such as cobalt glass) but it is preferred, in accordance with the invention, to more accurately adjust the same by the addition of supplementary absorptive dyes. To this end it is found that rose 55 bengal selectively absorbs light in the region 530-580; and that acid magenta selectively absorbs light in the region 580-620. These two dyes, therefore, are especially effective to absorb light in the zones which are thus rendered 60 sensitive by the erythrosine, and hence to adjust the relief produced in the exposed film by light in these spectral zones independently and additively, and thus to control the height of the relief (or density) of the silver negative and the 65 gamma of the positive produced therefrom, to accord with the density or relief, and gamma produced in the blue zone, for example. It is to be observed that in the spectral zone F' (to which the emulsion is sensitive without erythrosine) the tartrazine is strongly absorptive. This results in confining the penetration of this component of the exposure light to low values and particularly to the region of lower relief contours. The relief contours in this region will, 75

however, be directly related to the intensity of this component of the exposure light and hence possess accurate proportionality and take up and transfer proportional amounts or concentrations 5 of dye to a printed blank, by imbibition, and especially to reproduce sharper contrasts in the lower range of intensities.

In the spectral zone made sensitive by the erythrosine (F') the sensitivity may be unnecessarily great in comparison to the sensitivity 10 of the silver salt as limited by tartrazine. Of this zone, the spectral component of the exposure light in the lower portion may be sharply absorbed by rose bengal, while that in the higher portion may be (less sharply) absorbed by acid magenta and allowed to penetrate still more deeply into the film. In both portions of this sensitized zone the contrast gradation or gamma (relative depths of penetration or thickness of 15 relief) will be proportionate to the intensities of the respective components of the exposure light, and controlled by the specific ratio of sensitivity to absorption, with respect to the exposure light intensity of each given wave length or spectral zone.

In accordance with the invention a gelatine emulsion sensitive to blue, blue-green, green and yellow light may be prepared in the customary manner, (as by treating a silver halide emulsion 30 with erythrosine or other sensitizing agent equivalent to erythrosine) by procedures well known in the art, to which may be added the several reagents above mentioned, as follows:

|              | Grams |
|--------------|-------|
| 35 Gelatine  | 100   |
| Tartrazine   | 10    |
| Rose bengal  | 0.750 |
| Acid magenta | 0.125 |

40 A transparent film is then coated with the emulsion and allowed to dry, when it is ready for use in the customary manner. The film may then be exposed, for example, through a suitable negative to light having a spectral range corresponding to the aggregate spectral range of absorption of the composite dye—or to the spectral range of sensitivity of the film, and then converted into a relief image, as for example in accordance with my Patent 1,535,700. Likewise 45 the exposed stock may be developed in any of the usual non-tanning development solutions, and, if desired, fixed in the usual way with hypo.

50 The resulting silver image may then be converted into a gelatin relief image, as by bleaching in a solution of ammonium dichromate and potassium bromide, sulphuric acid and water, or in a solution of chromic acid, sodium chloride and water, or potassium dichromate and hydrochloric acid, or potassium ferricyanide, dichromate, copper sulfate, and hydrochloric acid.

55 These solutions cause hardening of the gelatin in those parts of the film which contain silver, and permit the removal of the unhardened gelatin with hot water. Subsequent treatment with hypo followed by washing and drying, completes the operation of producing a gelatin relief image.

60 In the resulting relief images, in whatever suitable way adapted for developing them, the thicknesses and contours produced by the normal (silver sensitive) spectral region of the exposure light are low due to the absorption effect of the tartrazine, the contours of the middle portion (lower erythrosine sensitized) region are intermediate and controlled by the absorption effect 65 of the rose bengal, while the upper (erythrosine

sensitized) region which, per se, might be too high, is controlled by the relative absorption effect of the acid magenta.

The relief image thus obtained is eminently suitable for use in imbibition printing, and serves to produce an accurate printed image, in which the proper contrasts are reproduced throughout the entire range of intensities of the exposure light,—and the range of such contrasts is much greater than has heretofore been obtainable by 10 procedures or compositions of the prior art. Moreover, any specific variations which may be encountered (due to the dye employed, the film blank to be printed, etc.) in the low, medium or high region of light intensities may be several- 15 ly corrected, without affecting the other and correctly reproduced regions.

I claim:

1. In the art of reproducing photographic records, the method of controlling the exposure 20 density relation of film prints which comprises sensitizing an emulsion for light including a wave length range of at least approximately 120 millimicrons, making said emulsion absorptive of light of at least three substantial wave length 25 zones substantially covering said range, the degrees of light absorption for the respective zones being stepped so that exposure light of said range penetrates to three substantial depths corresponding to said zones stepped throughout the 30 emulsion, printing on said emulsion with light including said range and adjusting the exposure density relation of each zone through absorption of the emulsion and exposure light intensity, thereby controlling the exposures of said zones 35 substantially independently and thus adjusting the shape of the total density exposure relation.

2. In the art of reproducing photographic records, the method of controlling the exposure density relation of film prints which comprises 40 rendering an emulsion throughout its depth sensitive to, and absorptive of, three substantial wave length zones representing together a spectral range of at least approximately 120 millimicrons, said sensitivity and absorption being 45 stepped for said three zones so that exposure light of said range penetrates to three substantial depths corresponding to said zones stepped throughout the emulsion, printing on said emulsion with light including said range and adjusting 50 the exposure of each zone with sensitivity and absorption of the emulsion and exposure light intensity, thereby substantially independently controlling the exposures of said zones and thus adjusting the shape of the total density exposure relation.

3. In the art of reproducing photographic records, the method of controlling the exposure density relation of film prints which comprises rendering an emulsion throughout its depth 60 sensitive to, and absorptive of, three distinct substantial wave length zones representing together a spectral range of at least approximately 120 millimicrons, said sensitivity and absorption being stepped for said three zones so that exposure 65 light of said range penetrates to three substantial depths corresponding to said zones throughout the emulsion, printing on said emulsion with light of said range and independently adjusting the exposure-density relation of each zone 70 by adjusting the intensity of its exposure light, thereby substantially independently controlling the exposures of said zones and thus adjusting the shape of the total density exposure relation.

4. In the art of reproducing photographic rec- 75

ords, the method of controlling the exposure density relation of film prints which comprises sensitizing an emulsion throughout its depth for light including a wave length range representing at least approximately 120 millimicrons, making said emulsion throughout its depth absorptive of light of at least three substantial wave length zones substantially covering said range by incorporating therein three dyes acting as filters absorbing light of wave lengths of said zones, the degrees of absorption for the respective zones being stepped so that exposure light of wave lengths of said range penetrates to three substantial depths corresponding to said zones stepped throughout the emulsion, printing on said emulsion with light including said range, and controlling the configuration of the density exposure relation for each zone and depth substantially independently by adjusting sensitivity and absorption of the emulsion and exposure light intensity, thereby controlling the shape of the total density exposure relation.

5. Reproduction film comprising an emulsion sensitized throughout for light including a wave length range of at least approximately 120 millimicrons, and at least three dyes acting as filters incorporated throughout the emulsion, said dyes absorbing light of at least three substantial wave length zones substantially covering said range, the light absorption degree of said dyes being stepped for penetration of light of the wave lengths of said zones to three substantial depths corresponding to said zones stepped throughout the emulsion.

35 6. Reproduction film comprising an emulsion sensitized throughout for approximately the blue, green and yellow wave lengths, and dyes acting as filters incorporated throughout the emulsion, said dyes absorbing blue, green and yellow light, the respective light absorption degree of said dyes being stepped for penetration of blue, green and yellow light, respectively, to three substantial depths corresponding to said zones stepped throughout the emulsion.

45 7. The method of making reproduction film which comprises sensitizing the film emulsion for light including a wave length range of at least approximately 120 millimicrons, and treating the same with at least three dyes selectively absorptive of light of at least three substantial wave length zones substantially covering said range, the degrees of light absorption of said dyes being stepped so that exposure light of said range penetrates to three substantial depths corresponding to said zones stepped throughout the emulsion.

8. The method of making reproduction film which comprises rendering its emulsion throughout its depth sensitive for a wave length range of at least approximately 120 millimicrons, and incorporating therein, substantially throughout its depth, at least three dyes acting as filters, said dyes absorbing light of at least three substantial wave length zones substantially covering said range, the light absorption degree of said dyes being stepped for penetration of light of the wave lengths of said zones to three substantial depths corresponding to said zones stepped throughout the emulsion.

70 9. The method of making reproduction film, which comprises the steps of rendering the film emulsion sensitive to all of the spectral zones of white exposure light and treating the same with three dyes, said dyes being selectively absorptive of light in the ultra violet to blue zone, in the blue

green to greenish yellow zone, and in the yellow-red zone, respectively, of the white exposure light, said selective absorption being stepped for the penetration of the exposure light of wave lengths of the respective zones to three substantial depths corresponding to said zones throughout the emulsion. 5

10. The method of making light sensitive film, which comprises the steps of rendering the film emulsion sensitive to all of the spectral zones of white exposure light, and treating the same with three dyes, one being selectively and strongly absorptive of light in the ultra violet to blue zone, the second being selectively and moderately absorptive of light in the blue green to greenish yellow zone, and the third being selectively and slightly absorptive of light in the yellow to red zone, of the white exposure light.

11. The method of making matrix film suitable for imbibition printing, which comprises the steps of rendering the same sensitive to all of the spectral zones of white exposure light and treating the same with three dyes, said dyes being selectively absorptive of light in the ultra violet to blue zone, in the blue green to greenish yellow zone, and in the yellow-red zone, respectively, of the white exposure light, said selective absorption being stepped for the penetration of the exposure light of wave lengths of said zones to three substantial depths corresponding to said zones throughout the emulsion, subjecting the emulsion to exposure light of varying intensities containing the wave lengths of said zones, developing the exposed film, and removing the undeveloped portions of the emulsion. 35

12. The method of making matrix film suitable for imbibition printing, which comprises the steps of rendering the film emulsion sensitive to all of the spectral zones of white exposure light, and treating the same with three dyes, one being selectively and strongly absorptive of light in the ultra violet to blue zone, the second being selectively and moderately absorptive of light in the blue green to greenish yellow zone, and the third being selectively and slightly absorptive of light in the yellow to red zone, of the white exposure light, subjecting the emulsion to white exposure light of varying intensities, developing the exposed film and removing the undeveloped portions of the emulsion. 50

13. Method of making photographic emulsion for the development of a wide range of contrasts therein comprising sensitizing the same with a silver salt and with erythrosine, and rendering the same selectively absorptive with respect to light of shorter wave length zone, to produce low contrast gradients in the normally sensitive region, rendering the emulsion selectively absorptive with respect to light of intermediate wave length to produce an intermediate region of densities or contrast gradient contours corresponding to the lower erythrosine sensitized zone, and rendering the emulsion selectively absorptive with respect to light of longer wave length, to produce the higher contrast gradient in the region of greater densities corresponding to the upper erythrosine sensitized zone. 55

14. Method of making photographic emulsion for the development of a wide range of contrasts therein comprising sensitizing the same with a silver salt and with erythrosine, and rendering the same selectively absorptive with respect to the zone of light of short wave length, by the addition of tartrazine to produce low densities or contours in the normally sensitive region, ren- 75

dering the emulsion selectively absorptive with respect to light of intermediate wave length to produce an intermediate density or contours region corresponding to the lower erythrosine sensitized zone, by the addition of rose bengal, and rendering the emulsion selectively absorptive with respect to light of longer wave length, to produce the higher density or contours region, corresponding to the upper erythrosine sensitized zone by the addition of acid magenta.

15. Method of making photographic emulsion for the development of a wide range of contrasts therein comprising sensitizing the same with a silver salt and with rose bengal, and rendering the same selectively absorptive with respect to

the zone of light of short wave length, by the addition of tartrazine to produce low densities or contours in the normally sensitive region, rendering the emulsion selectively absorptive with respect to light of intermediate wave length to produce an intermediate density or contours region corresponding to the lower rose bengal sensitized zone, by the addition of rose bengal, and rendering the emulsion selectively absorptive with respect to light of longer wave length, to produce 10 the higher density or contours region, corresponding to the upper sensitized zone by the addition of acid magenta.

LEONARD T. TROLAND. 15